

# UNITED STATES PATENT OFFICE

ALFRED L. PELLEGRIN, OF TUCSON, ARIZONA.

## PROCESS OF TREATING ORES.

1,233,398.

Specification of Letters Patent. Patented July 17, 1917.

No Drawing.

Application filed November 13, 1916. Serial No. 131,015.

To all whom it may concern:

Be it known that I, ALFRED L. PELLEGRIN, a citizen of the United States, residing at Tucson, in the county of Pima and State of 5 Arizona, have invented a certain new and useful Improvement in Processes of Treating Ores, of which the following is a full, clear, and exact description.

This invention relates to processes of separating ores; and it comprises a method of treating ores containing mineralized heavy metal salts of the oxidized heavy metal acids such as the lead salts by taking advantage of the differential attack upon the crystals or particles of such salts by sulfureted hydrogen, sulfids and the like with a preferential flotation of the attacked particles; and it more particularly comprises a method of recovering vanadates of lead from mixed 20 ores containing such vanadates and other lead salts, and in particular lead molybdate; all as more fully hereinafter set forth and as claimed.

Vanadium being now in great demand 25 there is an active search for ores containing this metal. Among the more valuable ores are lead ores containing lead vanadate. These ores, however, as a rule, are rather poor and they always contain many other 30 lead salts than the vanadate. Some contain in addition to the vanadate the molybdate of lead (wulfenite). It is of course comparatively easy to separate the lead minerals from the rest of the gangue because 35 of the great specific gravity of these lead minerals in general; but it is less easy to separate the lead minerals from each other, since their specific gravity is much the same. It is particularly difficult to separate van- 40 date of lead from the molybdate of lead where they occur in the same ore. Separately these two lead minerals are of considerable value; but in admixture they are of little value.

45 I have discovered that I can make a preferential separation of these various lead minerals from each other by the simple expedient of selectively sulfidizing their surfaces in a plurality of stages and then sub- 50 mitting them after each stage to flotation with oil and agitation in the usual way. These lead minerals being of oxidized nature are of course not susceptible of flotation with oil in their natural state, but become so sus- 55 ceptible when superficially converted into sulfids. If all the various minerals were

converted into sulfids superficially no separation would of course be possible by flotation; but I have found that these various lead minerals when exposed to the action of 60 a limited amount of sulfureted hydrogen, of sodium sulfid, etc., are not all attacked at the same rate. The action of the sulfur is preferential. And I find that by proper regulation of conditions with an ore containing 65 lead carbonate, lead oxid and other lead salts together with lead vanadate, the lead vanadate is the last to be attacked by sulfur compounds. Therefore in any such mixture by applying a suitable amount of a sulfur 70 reagent, the amount being such that the vanadate is not attacked, and then floating with oil and agitation in the usual way, the other lead minerals may be floated and thereby separated from the lead vanadate. If 75 the mineral also contains lead molybdate, on treatment with a small amount of sulfur as before in the flotation, the lead vanadate and lead molybdate will be left in the residue. On again preferentially sulfidizing, 80 the lead molybdate may now be floated leaving the lead vanadates as a residue. In other words, by performing the sulfidizing and flotation in successive steps, I can separate such a complex lead ore into a plurality 85 of different mineral products of good commercial grade.

In a practical embodiment of the present invention treating a highly complex ore carrying lead carbonate, lead oxid, lead molyb- 90 date and lead vanadate together with gangue, I first treat the ore in any of the usual ways and by any of the usual methods of concentration, wet or dry, to separate the gangue and to make a concentrate consist- 95 ing of the stated lead minerals. If the amount of gangue is inconsiderable this preliminary treatment may of course not be necessary. As a rule grinding should be carried only so far that distinct crystal faces 100 of the minerals to be separated still exist.

Having the pure concentrates in a wet condition, I may next blow sulfureted hydrogen through the pulp; or I may mix a little sodium sulfid in solution with such pulp. 105 In either event sulfidizing is stopped as soon as the mineral which is desired to float is attacked and before the other minerals exhibit signs of action. The mixture is now treated with oil and water and agitated in 110 the usual way, giving a float of the attacked lead particles. In the particular ore here

mentioned I ordinarily float the lead carbonate and oxid together. This now leaves me a residue containing lead molybdate and lead vanadate. As stated, the mixture of these two minerals is worth very little, but severally they are very valuable. This residue I again sulfidize, ceasing the treatment before the particles of lead vanadate are materially affected. On now adding oil and water and agitating the wulfenite or lead molybdate may be selectively floated, leaving the lead vanadate in the residue as a material of commercial grade.

Any suitable oil or process of flotation may be applied in the flotation operation and any suitable apparatus may be employed. In the preliminary concentration of the ore any ordinary method may be used.

Having thus described my invention, what I claim is:

1. In the separation of lead vanadate from other lead minerals the process which comprises sulfidizing the surfaces of particles of such other lead minerals, discontinuing the treatment prior to substantial attack of the vanadate and then separating the attacked mineral from the lead vanadate by flotation.

2. In the separation of lead salts of heavy metal acids from other lead minerals in a lead ore, the process which comprises sulfidizing the surfaces of such other minerals, discontinuing the sulfidizing prior to the attack on the particles of the lead salts of such heavy metal acids and subjecting the mixture to flotation to remove the attacked particles.

3. In the separation of lead molybdate and lead vanadate from other lead minerals in complex ores containing the same, the process which comprises submitting the ore mixture to a sulfidizing treatment until the surfaces of the particles of such other lead minerals are attacked, submitting to flotation to remove the attacked particles, again sulfidizing the residue to such an extent as to attack the lead molybdate only and subjecting the mixture to flotation to obtain the lead molybdate as floats and lead vanadate as a residue.

In testimony whereof, I hereunto affix my signature in the presence of two witnesses.

ALFRED L. PELLEGRIN.

Witnesses:

PAUL GATLIN,  
M. GATLIN.